



US011742162B2

(12) **United States Patent**  
**Best et al.**

(10) **Patent No.:** **US 11,742,162 B2**  
(45) **Date of Patent:** **Aug. 29, 2023**

- (54) **PHASE CHANGE NANO ELECTRO-MECHANICAL RELAY**
- (71) Applicant: **CARNEGIE MELLON UNIVERSITY**, Pittsburgh, PA (US)
- (72) Inventors: **James Best**, Pittsburgh, PA (US); **Gianluca Piazza**, Pittsburgh, PA (US)
- (73) Assignee: **Carnegie Mellon University**, Pittsburgh, PA (US)
- (\*) Notice: Subject to any disclaimer, the term of this patent is extended or adjusted under 35 U.S.C. 154(b) by 57 days.

- (21) Appl. No.: **17/294,906**
- (22) PCT Filed: **Dec. 18, 2019**
- (86) PCT No.: **PCT/US2019/067128**  
§ 371 (c)(1),  
(2) Date: **May 18, 2021**
- (87) PCT Pub. No.: **WO2020/132037**  
PCT Pub. Date: **Jun. 25, 2020**

(65) **Prior Publication Data**  
US 2022/0020545 A1 Jan. 20, 2022

**Related U.S. Application Data**

- (60) Provisional application No. 62/917,630, filed on Dec. 19, 2018.
- (51) **Int. Cl.**  
**H01H 37/36** (2006.01)  
**H01H 1/00** (2006.01)
- (52) **U.S. Cl.**  
CPC ..... **H01H 37/36** (2013.01); **H01H 1/0094** (2013.01); **H01H 2300/036** (2013.01)

- (58) **Field of Classification Search**  
CPC . H01H 37/36; H01H 1/0094; H01H 2300/036  
(Continued)

(56) **References Cited**

**U.S. PATENT DOCUMENTS**

- 5,903,099 A 5/1999 Johnson et al.  
7,755,899 B2 \* 7/2010 Stenmark ..... H01H 37/36  
337/393

(Continued)

**OTHER PUBLICATIONS**

International Search Report and Written Opinion for International Patent Application No. PCT/US2019/067128 dated Jun. 2, 2020, 10 pages.

(Continued)

*Primary Examiner* — Anatoly Vortman

(74) *Attorney, Agent, or Firm* — KDW Firm PLLC

(57) **ABSTRACT**

A MEMS/NEMS actuator based on a phase change material is described in which the volumetric change observed when the phase change material changes from a crystalline phase to an amorphous phase is used to effectuate motion in the device. The phase change material may be changed from crystalline phase to amorphous phase by heating with a heater or by passing current directly through the phase change material, and thereafter quenched quickly by dissipating heat into a substrate. The phase change material may be changed from the amorphous phase to a crystalline phase by heating at a lower temperature. An application of the actuator is described to fabricate a phase change nano relay in which the volumetric expansion of the actuator is used to push a contact across an airgap to bring it into contact with a source/drain.

**12 Claims, 9 Drawing Sheets**



(58) **Field of Classification Search**

USPC ..... 337/298  
See application file for complete search history.

(56)

**References Cited**

## U.S. PATENT DOCUMENTS

9,368,720 B1 \* 6/2016 Moon ..... H01L 45/16  
2009/0040007 A1 2/2009 Stenmark  
2009/0278111 A1 \* 11/2009 Pop ..... G11C 13/0004  
257/4  
2011/0038093 A1 \* 2/2011 Furukawa ..... H01G 5/18  
257/3  
2014/0264230 A1 \* 9/2014 Borodulin ..... H01L 45/1226  
257/4  
2014/0266300 A1 \* 9/2014 Sherwin ..... H03K 19/1736  
326/38  
2016/0035973 A1 \* 2/2016 Raieszadeh ..... H01L 45/1206  
257/4

2016/0079019 A1 \* 3/2016 Borodulin ..... H01H 37/46  
337/396  
2016/0172113 A1 \* 6/2016 Reig ..... H01G 4/33  
361/278

## OTHER PUBLICATIONS

Zhou et al., "A Zero Density Change Phase Change Memory Material: GeTe—O Structural Characteristics Upon Crystallization", Scientific Reports, vol. 5, Article No. 11150, Published Online Jun. 11, 2015, 13 pages.

Author Unknown, "Chalcogenide Glass", Wikipedia [online], Published on Oct. 10, 2018, Retrieved on Mar. 31, 2020, 4 pages.

Wang et al., "Directly Heated Four Terminal Phase Change Switches", 2014 IEEE MTT-S International Microwave Symposium (IMS2014), Jun. 1-6, 2014, 4 pages.

\* cited by examiner



FIG. 1



**FIG. 2A**



**FIG. 2B**



**FIG. 2C**



**FIG. 2D**



Amorphous

FIG. 3A



Height Change ↓

FIG. 3B



Crystalline

FIG. 3C



FIG. 3D



FIG. 4



1. Off  
Crystalline phase  
Contact does not touch d/s

**FIG. 5A**



2. Switching  
Joule heating of heater  
Melts pc material

**FIG. 5B**



3. On  
Quench in amorphous phase  
Contact touches d/s

**FIG. 5C**



4. On  
Amorphous phase  
Contact touches d/s

**FIG. 6A**



5. Switching  
Joule heating of heater  
Heats pc material

**FIG. 6B**



6. Off  
Converts to crystalline phase  
Contact does not touch d/s

**FIG. 6C**



FIG. 7





FIG. 8F



FIG. 8G



FIG. 8H

**PHASE CHANGE NANO  
ELECTRO-MECHANICAL RELAY**

**RELATED APPLICATIONS**

This application is a national phase filing under 35 U.S.C. § 371 claiming the benefit of and priority to International Patent Application No. PCT/US2019/067128, filed on Dec. 18, 2019, which claims benefit of U.S. Provisional Patent Application No. 62/917,630, filed on Dec. 19, 2018. The entire contents of these applications are incorporated herein by reference.

**BACKGROUND OF THE INVENTION**

Semiconductor-based materials, such as vanadium oxide ( $\text{VO}_2$ ), have been used for the synthesis of very high work density actuators by exploiting thermally-induced phase change transformation. Germanium Telluride (GeTe) is a phase change material that can be transitioned from a crystalline phase to an amorphous phase when heated to  $\sim 1000^\circ \text{ K}$  (sufficient to melt the material) and quickly quenched. The transition to the amorphous phase results in a volumetric increase of about 10%. This transition is reversible in nature, as the material undergoes a transition from an amorphous phase to a crystalline phase upon heating to  $\sim 500^\circ \text{ K}$ , resulting in a decrease in volume of the material

**SUMMARY OF THE INVENTION**

GeTe, as a semiconductor material with one of the largest work densities, is used herein for the making of micro/nanoscale actuators based on a volumetric change resulting from a transition from a crystalline phase to an amorphous phase and back to a crystalline phase. The change in volume of the material when undergoing a phase transition can be used to fabricate micro/nanoscale actuators, which can be used to fabricate micro/nano relays and other devices. Different from any other phase change material, GeTe is inherently non-volatile, making it of particular interest for applications in MEMS/NEMS relays or micro/nano robotics.

**BRIEF DESCRIPTION OF THE DRAWINGS**

FIG. 1 is a SEM image of a GeTe phase-change actuator.

FIG. 2 shows a fabrication flow for a phase change mechanical actuator.

FIG. 3 is an optical microscope image of a fabricated device showing the phase change material in both amorphous and crystalline phases.

FIG. 4 shows multiple actuation cycles of a phase change NEMS actuator showing the differences in height above the heater of the phase change material between the amorphous and crystalline phases.

FIG. 5 is a schematic representation of the steps to turn a first embodiment of a NEMS relay from an off state to an on state.

FIG. 6 is a schematic representation of the steps to turn the first embodiment of the NEMS relay from an on state to an off state.

FIG. 7 is a schematic representation of the steps to turn a second embodiment of a NEMS relay from an off state to an on state and back to the off state.

FIG. 8 is a schematic representation of the steps to fabricate the first embodiment of the NEMS relay.

**DETAILED DESCRIPTION**

5 A phase change MEMS actuator is shown in FIG. 1 and consists of three main components: the heater, phase change material (PCM), and cap. The heater is a thin wire capable of rapidly reaching the melting temperature of the PCM. The 10 PCM sits on top of the heater, isolated by a thin insulator to prevent current from flowing within the PCM. The cap is a thin insulator that protects the PCM from the atmosphere and reduces reflow of the PCM when in the liquid state. The device is switched by pulses through the heater. One heater 15 electrode is held at ground while square voltage pulses or another voltage waveform is applied to the other electrode. The PCM is converted to the amorphous (volumetrically larger) state by melting and quenching the material. Quenching must be fast enough to prevent crystallization from 20 occurring within the heated area. This can be accomplished by rapidly dissipating heat into the substrate. The PCM is converted back to the crystalline (volumetrically smaller) state by heating the material to promote rapid crystallization.

The phase change materials for the actuator may be 25 chalcogenide glasses (e.g. GeTe, GeSbTe, and other compounds), perovskite nickelates (e.g.  $\text{NdNiO}_3$ ,  $\text{SmNiO}_3$ ) or more generally rare earth perovskites,  $\text{RNiO}_3$  (where R=rare earth). The heater, contact metals, source and drain may be 30 any metal, any refractory material (e.g. W, Mo, Ru etc.), conductive oxides (e.g.  $\text{RuO}_2$ ,  $\text{TaO}_2$ ) or conductive nitrides ( $\text{TiN}$ ,  $\text{TaN}$ ).

In a preferred embodiment of the invention, the phase change material is GeTe. In one embodiment, the actuator may have the following dimensions: thickness: 200 nm, 35 width: 5.5  $\mu\text{m}$ , length: 15  $\mu\text{m}$ . The actuator may be fabricated on a substrate of AlN on Si having a thickness of approximately 100 nm. The heater may be composed of W and may have the following dimensions: thickness: 50 nm, width: 1.5  $\mu\text{m}$ , length: 11  $\mu\text{m}$ . The 816 may be composed of 40 an insulator, for example  $\text{Al}_2\text{O}_3$ , and may be approximately 20 nm in thickness. It should be realized that the dimensions provided are exemplary only and that the dimensions of the components of the actuator may vary based on application, fabrication method and chosen materials.

45 In an alternate embodiment of the invention, the phase change material may be conductive and the transition between phases can be accomplished by applying a voltage to the phase change material.

An exemplary phase change actuator may be fabricated 50 following the process shown in FIG. 2. As shown in View (A), fabrication starts on a silicon wafer 202. Wafer 202 is initially patterned and etched with alignment marks for future lithography steps. Wafer 202 is then coated with a 100 nm aluminum nitride (AlN) isolation layer 204. The AlN 55 layer 204 is compatible with subsequent high temperature processes and acts as an etch stop when patterning the heater. The AlN layer 204 is highly thermally conductive, ensuring the GeTe can be quenched in the amorphous state. Next, the heater 206 is added by depositing a layer of tungsten by sputtering at an elevated substrate temperature of 60  $850^\circ \text{ C}$ . The high substrate temperature during deposition is needed to deposit low resistivity tungsten, which is required for high-reliability heaters. The heater 206 is then patterned by an  $\text{SF}_6$  reactive ion etch, stopping on the base 65 AlN layer 204. Next, as shown in View (B), a conformal first insulating layer 208 of 10 nm thick  $\text{Al}_2\text{O}_3$  is deposited by atomic layer deposition (ALD). The first insulating layer 208

is needed to prevent joule heating in the GeTe 210. Without this layer, the melted portion of GeTe 210 is not contained by solid GeTe 210, which may result in a “blow out.” Next, GeTe 210 is deposited by co-sputtering Ge and Te at an elevated substrate temperature of 400° C. The elevated substrate temperature is required to ensure the deposited GeTe 210 is in the crystalline state. As shown in View (C), the GeTe 210 is then patterned by an Ar plasma etch, stopping on the first insulating layer 208. Finally, the GeTe 210 is encapsulated in a second insulating layer 212 of 20 nm of Al<sub>2</sub>O<sub>3</sub> deposited by ALD.

The device may be actuated using a 7 V 200 ns pulse to convert the PCM to the amorphous state, or a 6 V 200 ns pulse to convert the PCM back to the crystalline state. Other waveforms and voltages may be equally effective. FIG. 3 shows optical images of a device switching between amorphous and crystalline states. The optical properties of GeTe change depending on the crystal structure. As fabricated, the GeTe is in the crystalline phase. View (A) shows an actuated device. The dark area over the heater is the GeTe converted to the amorphous phase. This area, melted and quenched during the actuation pulse, is where the actuator expands, as shown in View (B). Converting back to the crystalline state removes this dark section of GeTe, as shown in View (C), and contracts the actuator, as shown in View (D).

FIG. 4 shows profile measurements of a device over three consecutive switching events. All measurements are referenced to the heater electrodes. The patterned GeTe rises above the heater. A height cross-section is taken down the length of the heater. Profile A is the as-fabricated actuator. All of the PCM is in the crystalline state, leading to a flat cross-sectional profile. When a 7 V 200 ns pulse is applied to the device, the device shifts from profile A to profile B. A section of PCM over the heater rises, matching the profile of amorphous material seen in the example optical measurements of FIG. 3. The cross-sectional profiles A and B show a height difference between the two states. An average height increase of 26 nm was measured over the actuated area.

When a 6 V 200 ns pulse is applied to the device, the device shifts from profile B to profile C. The amorphous section of PCM contracts back to the crystalline state. The cross-sectional profiles of B and C show a height difference between the amorphous and re-crystallized PCM. An average height decrease of 14 nm was measured over the actuated area, approximately 7% of the fabricated PCM thickness.

When a second 7 V 200 ns pulse is subsequently applied to the device, the device shifts from profile C to profile D. The previously actuated section of PCM again expands. The cross-sectional profiles of C and D show a height difference between the previously re-crystallized and the amorphous PCM. An average height increase of 16 nm was measured over the actuated area, approximately 8% of the fabricated PCM thickness.

The mechanical phase change actuator is able to expand and contract depending on the magnitude and length of the applied voltage pulses. Profiles of dark areas seen in the optical microscope images in FIG. 3 match those of the raised profiles shown in FIG. 4. The initial expansion of the actuator is larger than the subsequent contraction and expansions. Inconsistent or inadequate heating of the PCM, heater expansion, and reflow of the PCM are possible causes for this change in the magnitude of the expansion.

The PCM-based actuator is a new class of non-volatile MEMS actuator based on GeTe phase change material, which exhibits a large volumetric increase when converting from crystalline to amorphous phases. The demonstrated

actuator is capable of unidirectional strain up to 7% by confining the GeTe, allowing only expansion in the vertical direction. Phases are switched by pulsing a heater to melt and quench or heat the PCM to convert to the amorphous or crystalline phases respectively. Both amorphous and crystalline phases are stable at room temperature, making the actuator non-volatile. An average 14 nm thickness difference is achievable between amorphous and crystalline phases for a 200 nm thick GeTe actuator.

10 The actuator may have many practical applications in situations where movement is required in MEMS or NEMS devices. One such application is the fabrication of a phase change NEMS relay. The phase change NEMS Relay (PCNR) is a novel NEMS relay built on the phase change mechanical actuator previously described. The PCNR is actuated by the volumetric differences seen in the different phases of a phase change material. Some phase change materials, namely GeTe, have been observed to exhibit up to 15 a 10% volume change when switching between the amorphous (larger) and crystalline phases (smaller). These phases can be toggled by thermal cycling with the steps shown in FIG. 5.

View (A) of FIG. 5 shows the device in the “off” state, wherein the phase change actuator is in the crystalline phase.

25 The metallic contact is separated from the drain/source by an air gap and from the phase change actuator by a layer of insulating material. In View (B), the heater has been turned on by applying a pulsed voltage to the electrodes of the heater, thereby melting a portion of the phase change actuator, which is forced in the direction of the metallic contact by containment by the un-melted portion of the phase change material. The phase change material initially expands when melted, thereby pushing the metallic contact through the air gap, and forcing it against the drain/source. 30 The device is switched “on”. In View (C), the heater has been switched off and the phase change actuator is allowed to quench by having the heat quickly dissipate into the substrate via the highly-thermally-conductive AlN Layer. After quenching, the portion of the phase change actuator which was previously melted, as shown in View (B), is 35 locked in the expanded amorphous phase, thereby keeping the metallic contact pressed against drain/source. The device is now held “on”.

View (A) of FIG. 6 shows the device in the “on” state with

40 the metallic contact touching the drain/source. In View (B), the heater is switched on, heating the amorphous phase change actuator at a lower temperature than in View (B) of FIG. 5. This may be accomplished by applying a lower pulsed voltage or shorter pulse time to generate heat sufficient to transition the phase change material from the amorphous phase to the crystalline phase, but not sufficient to melt the material. In View (C), the phase change actuator is converted to a crystalline phase, which is smaller in size and does not push the metallic contact across the air gap into 45 contact with the drain/source. Because the air gap now separates the metallic contact from the drain/source, the device has been switched “off”.

An alternative “fin” geometry is shown toggling states in

50 FIG. 7. While built differently, both geometries use the same process to switch states. Expansion requires melting and rapidly quenching the material to change it to an amorphous phase. Contraction requires an elevated temperature, below the melting point, to facilitate a change to the crystalline phase in the material. The large volumetric change between 55 the two phases in the phase change material open and close air gaps for the PCNR. The phase change material also makes the device inherently non-volatile. As can be seen, the

phase change actuator is heated and pushes metallic contacts in a direction orthogonal to the substrate, where they push the metallic contact across the air gap into contact with the drain/source.

The PCNR is fabricated in an 8-step process, shown in FIG. 8. The first 4 steps are the similar to those in the previously described phase change mechanical actuator fabrication. In View (A), a silicon wafer 802 is initially patterned and etched with alignment marks for future lithography steps and coated with a 100 nm AlN isolation layer (not shown). The AlN is compatible with subsequent high temperature processes and acts as an etch stop when patterning the heater. The AlN is highly thermally conductive, ensuring the GeTe can be quenched in the amorphous phase. Next, heater 804 is deposited, comprising, in a preferred embodiment, a layer of tungsten (W) is deposited by sputtering at an elevated substrate temperature of 850° C. Other conductive materials may also be suitable from which to fabricate the heater. The high substrate temperature during deposition is needed to deposit the low resistivity tungsten required for high-reliability heaters. The heater is then patterned by an SF<sub>6</sub> reactive ion etch, stopping on the base AlN layer. Next, as shown in View (B), a conformal isolation layer 806 of 10 nm thick Al<sub>2</sub>O<sub>3</sub> is deposited by ALD. This layer is needed to prevent joule heating in the GeTe. Without this layer, the melted portion of GeTe cannot be contained by solid GeTe, which may result in a “blow out.” GeTe 808 is then deposited, as shown in View (C), by co-sputtering Ge and Te at an elevated substrate temperature of 400° C. The elevated substrate temperature is required to ensure the deposited GeTe is in the crystalline state. The GeTe 808 is then patterned by an Ar plasma etch, stopping on the Al<sub>2</sub>O<sub>3</sub> isolation layer. In View (D), the GeTe 808 is encapsulated in a layer of 20 nm of Al<sub>2</sub>O<sub>3</sub> 810 deposited by ALD.

After fabrication of the actuator, 30 nm of W is deposited and patterned, as shown in View (E), to form the metallic contact 812 for the switch. Next, 20 nm of SiO<sub>2</sub> is deposited by ALD as a sacrificial layer 814 and patterned with a CHF<sub>4</sub> plasma etch. This layer of oxide 814 is a sacrificial layer to set the air gap for the switch. In View (G), 500 nm of W is deposited and patterned to form the drain and source 816. The thick layer helps to mitigate changes in gap size caused by residual stress. Finally, the device is released by a vapor HF etch, removing the SiO<sub>2</sub> sacrificial material to form air gap 818.

An alternate embodiment of the PNCR may utilize the alternate embodiment of the actuator described above, in which the heater is eliminated and a voltage is applied directly to the phase change material to bring about the phase transition. In this case, the phase change material may be completely melted and will be contained by layer 810 of Al<sub>2</sub>O<sub>3</sub>.

As may be realized by one of skill in the art, the phase change actuator described herein can be utilized for many different applications, including the described phase change nano relay. Both the actuator and the phase change nano relay have been described in terms of the use of specific

materials and dimensions. It should be noted that the specific materials and dimensions are exemplary in nature and different combinations of materials and dimensions are possible without deviating from the intended scope of the invention.

We claim:

1. An actuator comprising:  
a substrate;  
an isolation layer, covering all or a portion of the substrate;  
a first insulating layer, covering all or a portion of the isolation layer;  
a phase change material, covering a portion of the first insulating layer; and  
a second insulating layer covering the phase change material;  
wherein the phase change material is encapsulated between the first and second insulating layers; and  
wherein a phase transition between a crystalline phase and an amorphous phase of the phase change material causes a movement of the second insulating layer.

2. The actuator of claim 1, the phase change material being transitioned from the crystalline phase to the amorphous phase by heating all or a portion of the phase change material at or above a melting point of the phase change material.

3. The actuator of claim 2, the phase change material being a conductive material, the phase change material changing phase by applying a voltage to the phase change material.

4. The actuator of claim 2, further comprising:  
a heater, disposed between the isolation layer and the first insulating layer, wherein the phase change material is heated by passing a current through the heater.

5. The actuator of claim 4, the heater comprising tungsten.

6. The actuator of claim 1, the phase change material being a chalcogenide glass, a perovskite nickelate or a rare earth perovskite.

7. The actuator of claim 6, the phase change material comprising GeTe.

8. The actuator of claim 2, the phase change material transitioning from the amorphous phase to the crystalline phase when heated to a second temperature, lower than the melting point.

9. The actuator of claim 8, the phase change material exhibiting a decrease in volume when changed from the amorphous phase to the crystalline phase.

10. The actuator of claim 1 wherein the first and second insulating layers are composed of Al<sub>2</sub>O<sub>3</sub> and the isolation layer is composed of aluminum nitride.

11. The actuator of claim 2 wherein the phase change material is transitioned to the amorphous phase by applying a 7 V 200 ns pulse to the phase change material.

12. The actuator of claim 2 wherein the phase change material is transitioned to the crystalline phase by applying a 6 V 200 ns pulse to the phase change material.

\* \* \* \* \*